

Patented Dec. 9, 1924.

1,519,085

# UNITED STATES PATENT OFFICE.

DAVID M. BARRY, OF BRISTOL, AND LAWRENCE C. HUMASON, OF FARMINGTON, CONNECTICUT, ASSIGNEES TO THE HUMASON MANUFACTURING COMPANY, OF FORESTVILLE, CONNECTICUT, A CORPORATION OF CONNECTICUT.

## METHOD OF ENAMELING COIL SPRINGS.

No Drawing.

Application filed December 23, 1921. Serial No. 524,543.

To all whom it may concern:

Be it known that we, DAVID M. BARRY and LAWRENCE C. HUMASON, citizens of the United States, and residents of Bristol and Farmington, respectively, county of Hartford, State of Connecticut, have invented 5 certain new and useful Improvements in Methods of Enameling Coil Springs, of which the following is specification.

10 In the process of enameling coil springs, the convolutions of which are normally close together, it is preferable to stretch the spring in order to uniformly apply the enamel and then bake the enamel on the 15 spring while the latter is in stretched condition to insure a uniform baking and an even coat. We have found, however, that the spring, when heated in a stretched condition to a temperature necessary to properly 20 bake the enamel, takes an objectional set, which tends to twist or distort the spring.

The aim of the present invention is to 25 provide an improved method of enameling wherein objectionable setting of the spring, resulting from baking the enamel while the spring is stretched, is prevented. To this end, the invention broadly contemplates initially heating the coil spring before applying 30 the enamel and while the spring is in its normal or unstretched condition to a temperature in excess to that at which it is necessary to bake the enamel on the spring but not sufficiently high to draw the 35 temper of the metal of the spring; then stretching the spring and applying the enamel thereon, and then baking the enamel while the spring is under tension. The temperature employed for initially heating the 40 coil spring will depend of course on the composition of the metal used in the spring. By proceeding in accordance with the method of the present invention, the enamel is effectively and evenly applied and baked, 45 insuring a neat, smooth finish and a rust-proof coating, and undue setting or twisting of the spring is effectively guarded against. The step of initially heating the coil spring before applying the enamel and while the 50 spring is in its normal or unstretched condition to a temperature in excess to that at which it is necessary to bake the enamel on the spring prevents objectionable setting of the spring which would otherwise result

during the operation of baking the enamel 55 while the spring is stretched.

The preferred method of procedure consists in heating the coiled wire in its normal condition (that is while it is not under tension or stretch) to a temperature higher 60 than that required for baking the enamel on the coil but not sufficiently high to draw the temper of the metal of the spring; then stretching the coil and applying the enamel 65 thereon in any suitable manner as by spraying or dipping; and then while the coil is stretched or extended, heating it until the enamel becomes tacky or set; then decreasing the extension or stretch of the spring 70 but still holding it under tension, and finally heating the spring in this condition, until the enamel becomes thoroughly hardened or baked, at a temperature less than that at which the spring was heated before the 75 enamel was applied, but greater than that employed for heating the spring until the enamel becomes tacky or set. If desired, the wire, after it has been initially heated and before the enamel is applied, may be subjected to a suitable rust-proofing process, 80 such as the Parkerizing process, but this is not necessary as the enamel itself will properly rust-proof the spring.

We have found that the method herein disclosed, while being susceptible of use in 85 enameling coil springs generally, has peculiar application in the enameling of a coil spring the convolutions of which are flattened or elongated, for instance such springs as are used as arm bands or garters. 90

We claim as our invention:—

1. That improvement in the art of enameling coil springs which consists in heating the coil spring in its normal condition, stretching said spring and applying the 95 enamel, and then baking the enamel on the spring while the latter is under tension.

2. That improvement in the art of enameling coil springs which consists in heating the coil spring in its normal condition to 100 a temperature higher than that necessary to bake the enamel on the spring, then stretching the spring and applying the enamel thereon, and then baking the enamel on the spring while the latter is under tension. 105

3. That improvement in the art of enameling coil springs which consists in heating

the spring to a temperature which will prevent setting of the spring when it is subsequently heated to bake enamel thereon, then applying the enamel with the spring in stretched condition and baking the enamel on the spring in stretched condition.

4. That improvement in the art of enameling coil springs which consists in heating the spring in its normal condition to a temperature higher than that required for baking enamel on the spring, applying enamel to the spring and heating the spring in

stretched condition until the enamel becomes tacky or set; then decreasing the stretch of the spring but still holding it under tension, 15 and finally heating the spring under tension at a temperature less than that at which the spring was heated before the enamel was applied but greater than that employed for heating the spring until the enamel became tacky or set. 20

DAVID M. BARRY.  
LAWRENCE C. HUMASON.